

A. H. MOORE.  
METHOD OF MAKING RAILWAY RAILS.  
APPLICATION FILED JAN. 4, 1913.

1,074,089.

Patented Sept. 23, 1913.

*Fig. 1.*



*Fig. 2.*



*Fig. 3.*



WITNESSES

Philip R. Hough  
J. H. Sherwood

INVENTOR

Alfred H. Moore,

Franklin D. Hough

BY

ATTORNEY

# UNITED STATES PATENT OFFICE.

ALFRED H. MOORE, OF NEW YORK, N. Y., ASSIGNOR OF ONE-HALF TO CHARLES F. MOLLEY, OF NEW YORK, N. Y.

## METHOD OF MAKING RAILWAY-RAILS.

1,074,089.

Specification of Letters Patent. Patented Sept. 23, 1913.

Continuation of application Serial No. 712,126, filed July 29, 1912. This application filed January 4, 1913. Serial No. 740,232.

*To all whom it may concern:*

Be it known that I, ALFRED H. MOORE, a citizen of the United States, residing at New York, in the county of New York and State of New York, have invented certain new and useful Improvements in Methods of Making Railway-Rails; and I do hereby declare the following to be a full, clear, and exact description of the invention, such as will enable others skilled in the art to which it appertains to make and use the same, reference being had to the accompanying drawings, and to the letters and figures of reference marked thereon, which form a part of this specification.

This invention relates to new and useful improvements in methods of making railway rails, the object being to produce a rail which will have great strength, affording great safety.

The invention consists further in the method of making rails of combination steel and iron, the combination being effected in a non-oxidizing atmosphere and consisting in a fusion of the metals, first forming an ingot with steel center and "best" iron envelop and afterward cutting the ingot in order to expose a steel surface which, when rolled, will form the tread or crown surface of the rail, while the "best" iron will form a continuous chair for the web and flange of the rail.

In carrying out my process reference is herein made to the accompanying drawings, in which:—

Figure 1 is a perspective view of an ingot having an inner core of steel and an envelop of "best" iron fused thereto, a portion of the ingot being shown in section. Fig. 2 is a detail view showing the ingot in section, and Fig. 3 is a perspective view of a rail rolled from one of the sections shown in Fig. 2 and having a tread surface of steel and a continuous chair and flange of "best" iron and fused to the steel core.

In making the rails in accordance with my method, an ingot, previously prepared

with an inner core of steel with a uniform percentage of carbon as may be desired to meet different conditions, is provided with an outer envelop of "best" iron fused thereto which is utilized by first cutting the ingot to expose a steel surface which, when the ingot is rolled into a rail, will form the crown or tread surface thereof. It will be understood that the original preparation of the ingot and its being cut and formed into a rail is done in the same heating. In heating the ingot, the envelop of "best" iron must be brought to a white heat and at which stage the steel forming the center will be in a semi-liquid or half molten condition. In this condition, the steel throws off carbon which consumes or destroys any of the phosphorus or sulfur contained in the iron, resulting in the production of an ingot equal and superior to the best charcoal iron with an appreciable gain in tensile strength. The ingot is then passed through the rolls with a gentle pressure so as not to burst the envelop and which will cure the steel of porosity. In the treatment of the ingot to cause the proper fusing of the iron and steel, the welding heat of wrought iron is 2700 degrees F., while steel melts at 2552 degrees F.

When the material of the ingot is in proper condition, it is severed longitudinally and centrally and the section of the ingot rolled by any suitable rolling mechanism in such a way that the severed surface will form the tread or crown of the rail while the "best" iron, which is fused to the steel core, will form a continuous chair or envelop for the web and flange of the rail.

A rail made in accordance with my method will have a hard tread surface.

This application is a continuation of an earlier application bearing Serial No. 712,126, filed July 29, 1912.

What I claim to be new is:—

The method of making railway rails consisting in taking an ingot having a steel center and "best" iron envelop fused to-

gether, severing the ingot longitudinally and centrally, then rolling the sectional ingots in such a manner that the steel will be exposed and will form the tread of the rail 5 and that the web and foot of the rail will have an outer surface of "best" iron and a core of steel.

In testimony whereof I hereunto affixed my signature in the presence of two witnesses.

ALFRED H. MOORE.

Witnesses:

A. L. HOUGH,  
FRANKLIN H. HOUGH.

Copies of this patent may be obtained for five cents each, by addressing the "Commissioner of Patents, Washington, D. C."